

March 30, 1926.

1,578,981

A. GELBERT

METHOD OF MAKING A LUSTROUS FABRIC

Original Filed April 29, 1921

Fig. 1.



Fig. 2.



Fig. 3.



Fig. 4.



Inventor:

Witness:

R. L. Harrington

Alfred Gelbert  
by Albert Scheibl,  
Attorney

Patented Mar. 30, 1926.

1,578,981

# UNITED STATES PATENT OFFICE.

ALFRED GELBERT, OF CHICAGO, ILLINOIS.

## METHOD OF MAKING A LUSTROUS FABRIC.

Application filed April 29, 1921, Serial No. 465,585. Renewed January 9, 1926.

To all whom it may concern:

Be it known that I, ALFRED GELBERT, citizen of the United States, residing at Chicago, Illinois, have invented certain new and useful Improvements in Methods of Making a Lustrous Fabric; and I do hereby declare the following to be a full, clear, and exact description of the invention, such as will enable others skilled in the art to which it appertains to make and use the same.

My invention relates to the production of new and highly useful materials from cheap fabrics and to the novel materials produced in this manner. Viewed in one general aspect, my invention aims to provide a handsome, inexpensive, flexible, waterproof and incombustible material adapted by its decided lustre to be used in place of silk or of other expensive materials. Furthermore, it aims to provide material of this kind embodying color effects combined with more or less lustre and having these color effects duly protected so as to protect them against humidity in the air and to permit the ready washing of the material. Furthermore, my invention aims to provide a simple and inexpensive process for producing lustrous and more or less translucent materials of this kind, for utilizing as the basis for such materials cheap fabrics such as cheese cloth, voile, calico or lace; for permitting the applying of suitable ornamentation in any desired colors to such a material at a certain stage during the process of its manufacture, and for suitably waterproofing the resulting colored or ornamented material.

In another aspect, my invention aims to use some single and simple chemical for simultaneously fireproofing a fabric and imparting a lustre to the same, and aims to treat the resulting fireproofed material in such a manner as simultaneously to waterproof the same and to reduce at least a portion of the fireproofing material to a crystalline condition in which it will reflect and refract light in imitation of silks or the like. Moreover, my invention aims to treat a previously fireproof fabric with a solution which will first dissolve at least a portion of the material with which the fabric was fireproofed and which will then solidify into a translucent coating holding crystallines of the previously dissolved fireproofing material suspended in the same.

Still further and more detailed objects will appear from the following specification

and from the accompanying drawings in which—

Fig. 1 is an enlarged cross-section of the initial cloth used in producing one embodiment of my invention, showing particles of the fireproofing and crystallizable material deposited on the same in the original non-crystalline form.

Fig. 2 is a similar cross-section of the same cloth after it has been subjected to the treatment which saturates and coats it with gelatin and which converts the fireproofing material into crystals incorporated in the gelatin.

Fig. 3 is a section similar to Fig. 2, showing the resulting lustrous material as mounted between two glass plates for use in imitation of stained or inlaid glass.

Fig. 4 is a fragmentary elevation of the imitation stained glass of Fig. 3, drawn on a smaller scale.

Generally speaking, I accomplish important purposes of my invention by saturating and coating the basic fabric with a solution of gelatin or the like after the fabric has been impregnated with a material which is adapted to form crystals, and by using for this impregnation a material which will be dissolved by the gelatin and which will crystallize within the latter so as to form a large number of crystals incorporated in the gelatin when the latter solidifies. For example, I may start by immersing a piece of cheese cloth or calico 1 in a solution composed of one ounce of calcium bromide dissolved in a quart of either alcohol or water, allowing the cloth to dry after it has been well soaked with this solution. This impregnation in itself would render the cloth non-combustible without materially altering its appearance, as the fireproofing compound 2 will be widely distributed over and through the cloth.

I then treat the impregnated (fireproofed) cloth with a gelatinous solution, such as that composed of two ounces of gelatin and one-half ounce of castor oil, dissolved in one quart of hot water. This gelatinous solution may be applied to the previously impregnated fabric either by immersing the latter in the same or by brushing the solution upon the cloth. In either case, the cloth is then allowed to dry, so as to permit the gelatin to harden into a translucent and more or less transparent coating 3 through which the fabric may be discerned. During

the treatment of the cloth in this hot gelatinous solution the calcium bromide, with which the cloth had been previously impregnated is dissolved in this solution, but 5 remains in substantially the same uniform distribution as that which it previously occupied and would therefore remain distributed over the cloth when the solution evaporates. However, owing to the difference between an ordinary aqueous solution 10 and a hot gelatinous solution, the calcium bromide crystallizes out of this solution and, owing to its fairly uniform distribution, will therefore form a large number of 15 relatively small crystals 4. While the resulting crystals may be too small to be readily discerned as such through the translucent coating of gelatin which covers both the cloth and the crystals when the gelatin 20 hardens, these crystals will readily reflect light from their flat faces. Consequently, when the resulting material is viewed in any strong light, a part of the light will be reflected from these widely scattered and 25 variously directed crystals 4, thereby imparting a sparkling or lustrous effect not found in ordinary gelatin-coated fabrics and in many ways resembling the lustre of silk.

30 If the resulting fabric is to be used for picture, window or sign effects the initially impregnated cloth is desirably stretched on a frame after it has been dipped into the bromide solution and is allowed to dry on 35 this frame. Then the hot gelatinous solution is brushed over the impregnated and dried cloth while still stretched and the gelatin-coated cloth is allowed to dry while on the frame, thereby affording a well stretched 40 surface to which any desired picture, wording or other artistic effect may be applied either with a brush or by some imprinting process. For example, any desired picture 45 may be painted on the surface of the gelatinous coating in water colors, and by using transparent colors for this purpose, the color effects will not interfere with the lustrous effect due to the crystals which are incorporated in the gelatin. Then by applying 50 a final coating of transparent lacquer or varnish, I can readily make the resulting material waterproof, so as to avoid having the color effects spoiled either by humidity in the air or by a washing of the finished 55 material.

For inlaid glass effects or the like I can proceed in a similar manner to that above described, but desirably use non-transparent colors for the division lines between the 60 mosaically arranged portions which correspond to the different colors of the glass pieces which I can readily imitate in this manner, that is to say, I employ transparent colors for the main glass effects 5 which are 65 to be reproduced and employ non-trans-

parent colors for the division lines 6 which imitate the lead joints. In this case, I may also employ water colors, as the final coating of varnish will readily prevent humidity from effecting the coloring. Then for imitation stained glass plates, I desirably enhance the resemblance still further by mounting the resulting lustrous fabric between a pair of clear glass plates 7 as shown in Fig. 3.

70 However, while I have heretofore mentioned certain materials as desirable in the production of fabrics according to my invention, I do not wish to be limited to the same, nor to the particular procedures above 80 outlined. For example, other crystallizable salts, such as sodium bromide may be used for the initial impregnation, and the desirable flexibility may be imparted to the gelatin by some non-volatile oil other than 85 castor oil, as for example rapeseed oil. Likewise, the fabric employed as the basic material may be greatly varied according to the nature of the desired product. Thus, 90 voile, calico, laces or other textile materials may be used for producing handsome effects. Nor do I wish to be limited to applying coloring with a brush, as this may be imprinted on the same, thereby permitting 95 the inexpensive production of such goods in large quantities.

Neither do I wish to be limited to the use of the resulting material for picture, sign or window effects, as it can readily be employed also for screens, lamp shades 100 and the like. Moreover, it can also be used for purposes where flexibility is essential, as for example for dress materials, window shades or the like. In other words, I aim 105 in the appended claims to cover all materials and methods of manufacture which come within the spirit of my invention.

110 I claim as my invention:

1. The process of producing a lustrous fabric which consists in treating an ordinary fabric with a solution of a crystallizable salt, drying the treated fabric, and then treating the dried fabric with a gelatinous solution.

115 2. The process of imparting lustre to a fabric which consists in treating the fabric with a solution of a crystallizable salt, drying the treated fabric, and then treating the dried fabric with a gelatinous solution including a non-vaporizing oil.

120 3. The process of producing a lustrous and fireproof fabric which consists in treating ordinary fabric with a solution of a fireproofing and crystallizable chemical, drying the treated fabric and thereafter treating the dried fabric with a hot gelatinous solution.

125 4. The process of producing lustre on a fabric which consists in impregnating the fabric with a crystallizable salt in a non-crystalline form and thereafter treating the 130

- impregnated fabric with a solvent for the said salt which will permit the salt to crystallize and which will form a translucent coating over the resulting crystals.
5. The process of producing lustre on a fabric which consists in impregnating the fabric with a crystallizable salt in a non-crystalline form, treating the impregnated fabric with an air-drying coating 15 adapted to dissolve the impregnating material under conditions which will cause the said solved material to crystallize within the said coating during the drying of the fabric with a hot gelatinous solution and latter.
10. drying the resulting gelatin coated fabric. Signed at Chicago, April 21st, 1921.
6. The process of producing lustre on a 20

ALFRED GELBERT.